

Jan. 5, 1932.

N. RASHEVSKY

1,840,130

THERMIONIC DEVICE

Filed May 27, 1926

Fig. 1.



Fig. 2.



WITNESSES:

*E. O. McElroy*

*H. H. Whittier*

INVENTOR  
*Nicolas Rashevsky*

BY  
*Hersey & Carr*  
ATTORNEY

## UNITED STATES PATENT OFFICE

NICOLAS RASHEVSKY, OF WILKINSBURG, PENNSYLVANIA, ASSIGNOR TO WESTINGHOUSE ELECTRIC & MANUFACTURING COMPANY, A CORPORATION OF PENNSYLVANIA

## THERMIONIC DEVICE

Application filed May 27, 1926. Serial No. 111,948.

My invention relates to vacuum tube devices and more particularly to such devices in which thermionic emission is obtained from a heated filament.

5 One of the principal objects of my invention is to produce a filament having high thermionic emissivity.

Another object is to produce a filament which will have a comparatively long life 10 and which may be manufactured at reduced cost.

Another object of my invention is to construct a filament which may be reproduced within fairly close limits so that tubes containing such filaments will have substantial- 15 ly uniform characteristics.

In the construction of cathodes, it is highly desirable that elements which have a low "work function" be used. This "work function" or, as it is sometimes known, "electron affinity", is expressed in terms of electrical potential or volts. The "work function"  $\phi$  is expressed in terms of Richardson's constant "D" by the relation:

$$25 \quad \phi = \frac{RD}{e} \times 300;$$

30 where R is the gas constant. The quantity  $\phi$  is one of the most important constants in thermionics, as on it depends the thermionic current which can be obtained from any particular type of cathode at any given temperature and is characteristic of the cathode substance.

35 The smaller we make  $\phi$ , the larger in general the thermionic current that can be obtained with a given cathode temperature. Consequently, a cathode having a low constant  $\phi$  will also tend to have a longer life, which is obviously desirable from the standpoint of economy. The thoriated cathode and the oxide coated cathode, now well known to those skilled in the art, are examples of 40 cathodes which have been so treated as to obtain a low value of "work function". These cathodes have not always proved entirely satisfactory in the past, in part due to the difficulty of making filaments having identical 45 properties and also to the fact that both types

have a limited life and are comparatively expensive to manufacture.

The present invention contemplates using, as a cathode, an element having a low-melt- 55 ing point which has also a low value of "work function". Among such elements, nickel seems to be one of the most desirable as it has a "work function" of 2.9 volts. Nickel, how- 60 ever, has a melting point which is too low to permit of it being used alone as a cathode 65 material since it would be subject to deformation long before the desired temperature is attained. The problem, then, was to discover some practical manner in which nickel or an analogous element could be used as a cathode 70 and could be prevented from deforming at the relatively high temperatures necessary to secure satisfactory electronic emission. This problem has been solved in an entirely 75 satisfactory manner by employing a highly refractory substance, such as tungsten or molybdenum for the filamentary or cathode base and then applying a coating of nickel or other metal having the desired characteristics.

I have used several different methods to provide the necessary coating to practice my invention. Among the preferred forms are electroplating, the decomposition of a nickel salt in place, or deposition of the nickel from the vaporized state. The latter method, which has given the best results, will be more clearly understood by reference to the dia- 80 grams.

85 Referring to the drawings which form a part of this application

Figure 1 shows one form of an apparatus for coating a filament or other cathode ele- 90 ment, and

Fig. 2 shows an alternative form.

In Fig. 1 is shown an evacuated container 1 having therein a properly mounted filament 2 of tungsten, or thoriated tungsten, a cylindrical anode 3 having a lead-in 4. Surrounding the container is a coil 5 suitably connected to a source of high frequency current 6, which may be an alternator, an oscil- 95 lation generator or an equivalent device. Although the anode is shown as a cylinder, any other convenient shape such as a plate 100

may be employed, and the filament is simply shown as indicative of a general class of articles to be coated.

In Fig. 2 is illustrated a tube having a plate 3, in lieu of the cylinder shown in Fig. 1, while the other elements numbered similarly to those of Fig. 1, correspond respectively thereto. The container comprising the nickel cylinder or plate, and the filament or other element to be coated, is first carefully exhausted to obviate any danger of the nickel oxidizing. The coil 5 is then supplied with high-frequency current, which induces in the cylinder or plate a sufficiently heavy current to raise its temperature to the point at which the nickel begins to vaporize.

This heating is continued until the interior of the receptacle 1 is coated and becomes, to a more or less degree, opaque. This deposit 20 on the tube walls is indicative that nickel has been thrown off from the cylinder or plate 3, and it has been found that the relative opacity of such deposit is a measure of the amount of nickel deposited on the filament as well. It is important that the filament be kept relatively cool during this operation, in order that the nickel will remain thereon after having been deposited, and this is accomplished much more readily when the apparatus of Fig. 2 is employed. In this view, the nickel element is shown as a plate, spaced several millimeters from the filament, which permits the filament to more efficiently radiate such heat as may be conveyed to it 30 from the plate than is the case with a tube as shown in Fig. 1. At the same time, it is obvious that less heat is transferred from such plate to the filament than when the cylinder entirely surrounds the filament.

It has not been found necessary to apply potential between elements 2 and 3 during this operation, the inductive heating of element 3 having been found sufficient.

A filament made according to my invention not only permits the use of nickel or an analogous element having a low melting point as a cathode material, but gives rise to an entirely unexpected high electron emission. It is my conclusion that this extremely high emission is due to the fact that by using my new type of filament, I am enabled to heat the nickel or other element above its melting point, so that during the operation of the filament, the nickel or other coating exists thereon in a closely adherent semi-liquid form. At the same time, it would appear probable that the "work function" of the coating material is also reduced.

It is also probable that the increased electronic emission is in some way related to the lowering of the surface tension of the melted metallic film but I am not, at this time, prepared to state exact reasons for this nor can I give a more exact theory of operation.

Another peculiar fact is noted in connection

with the use of my coated filaments; the film, although heated to a temperature above its melting point, is neither absorbed by the refractory carrier nor does it seem to amalgamate therewith.

I have also discovered that when nickel is applied to tungsten filaments having a trace of thorium oxide, the reduction of this oxide begins at a lower temperature than when nickel is not present. Accordingly, by using 75 a certain percentage of nickel with the well known thoriated filament, I am able to produce a cathode which is easier to activate, and which is extremely stable in operation.

It will thus be seen that I have produced 80 a cathode the characteristics of which are different in many respects from those so far known and used. My cathode has a very much higher electron emission than the usual type, has a longer life and is relatively cheaper to manufacture. Numerous advantages of 85 this type of cathode in addition to those enumerated will suggest themselves to those skilled in the art, and it is also, of course, obvious that many other combinations of refractory carrier and low-melting point coating 90 may be employed, all within the range of equivalents of my invention.

The essential feature of my invention which is broadly new and of greatest importance is the use as a cathode of an element having a comparatively low melting point and low "work function" so arranged and carried by a refractory material that it 95 may be heated above its melting point.

Although I have described herein only certain specific embodiments of my invention, it is not my intention to be limited thereby. No limitation except such as is necessitated by the prior art or expressed in the claims 100 is intended.

I claim as my invention:

1. The method of increasing the electron emissivity of a thoriated cathode which comprises vaporizing nickel in the presence of 110 said cathode until a thin coating of nickel is formed thereon.

2. In an electron-discharge device including a transparent vessel having a cathode of refractory material therein, the method of increasing the electron emission of said cathode which comprises vaporizing nickel within said container until said vessel becomes opaque, whereby a thin film of nickel 115 is formed on said cathode.

3. In an electron-discharge device including a transparent vessel having a cathode of refractory material therein, the method of increasing the electron emission of said cathode which comprises vaporizing nickel within said container while said cathode is unheated until said vessel becomes opaque, whereby a thin film of nickel is formed on 120 said cathode.

4. A cathode comprising a cathode of re- 125

fractory material having a thin film of nickel thereon, said film being in a semi-liquid form when the filament is heated to a temperature at which it freely emits electrons.

5 5. A cathode comprising a thoriated filament and a thin film of nickel adsorbed thereon.

6. A cathode comprising thorium and a thin nickel film adsorbed thereon.

10 7. A cathode comprising a tungsten element and a thin film of nickel, said film being held to said element by adsorption.

8. In a cathode, an element composed of a refractory conductive material, and a thin 15 film of nickel held thereon by adsorption.

9. A cathode comprising a refractory carrier having a layer of thorium thereon, and a thin film of nickel adsorbed on said thorium.

20 10. As a step in the method of activating a thoriated cathode, the adsorption of a thin nickel film thereon.

11. A cathode comprising a cathode of refractory material having a thin film of 25 nickel held by adsorption thereon, said film being not amalgamated with said material.

12. A cathode comprising a cathode of refractory material having a thin film of nickel held by adsorption thereon, said film being 30 not absorbed by said material.

In testimony whereof, I have hereunto sub-  
scribed my name this 21st day of May, 1926.

NICOLAS RASHEVSKY.

35

40

45

50

55

60

65